

## UNITED STATES PATENT OFFICE

2,085,014

## TEXTILE PROCESS AND PRODUCT

Camille Dreyfus, New York, N. Y., and William Whitehead, Cumberland, Md., assignors to Celanese Corporation of America, a corporation of Delaware

No Drawing. Application November 14, 1933,  
Serial No. 697,926. Renewed January 2, 1937

13 Claims. (Cl. 28—1)

This invention relates to textiles, films, etc. formed from a solution of a derivative of cellulose having incorporated therein an ingredient which does not adversely affect the solution from which filaments of good cross-section and better films may be formed. This application is a continuation-in-part of our application S. No. 318,583, filed November 10, 1928, which has issued as Patent No. 1,958,283.

10 An object of the invention is the production of improved artificial material bearing derivatives of cellulose as a basis. Another object of the invention is the production of improved staple fibres. Other objects will be apparent from the following description.

15 We have found that if yarns, filaments, films, foils or other artificial materials are formed from solutions of derivatives of cellulose containing wax-like bodies which are preferably emulsified in water the resulting product has many advantageous properties.

20 This invention is applicable to the formation of a yarn comprising substantially continuous filaments. It is of particular application to the formation of relatively short lengths or staples 25 which may be associated together by twisting to form "spun" yarn.

25 The yarn made according to this invention is easily delustered and forms a soft crinkly filament especially adapted to spinning as staple yarns, i. e. a yarn composed of twisted short filaments.

30 With our invention synthetic filaments can be spun to a crinkly fiber with a lower concentration of dope. In spinning filaments from cellulose acetate our invention permits the dry spinning of filaments of good cross-sections even at high concentrations of vapors of acetone or other solvent in the spinning cabinet.

35 The yarn spun according to our invention has a very slightly subdued lustre and an appearance more like that of real silk than normally spun yarn. A great advantage in our invention is that when yarn made according thereto is delustered 40 it becomes very woolly and crinkled and delusters very heavily.

45 This invention is applicable to the formation of yarns or filaments, under which terms are included, threads, assemblies or bundles of a number of continuous filaments which may be in parallel relationship or which may be twisted together, artificial bristles, straws, short lengths of staple fibres or yarn spun from such staple fibres. It is also applicable to the formation of other artificial products such as foils, films and the like.

This invention is particularly of importance in connection with the formation of artificial materials made of or containing organic derivatives of cellulose such as organic esters of cellulose and cellulose ethers. Examples of cellulose esters are cellulose acetate, cellulose formate, cellulose propionate and cellulose butyrate, while examples of cellulose ethers are ethyl cellulose, methyl cellulose and benzyl cellulose.

5 The yarns may have applied thereto or incorporated therein effect materials such as pigments, filling materials, dyes, lakes, etc., fire retardants such as beta chloronaphthalene, triphenyl phosphate or tricresyl phosphate either in a coating material or in the yarns or filaments or both.

10 We preferably incorporate in the spinning solution a wax-like body which is emulsifiable in water, soap solutions, solvents and like scouring baths. The wax-like body contains at least a 20 proportion of one or more such ingredients as mono-stearate of diethylene glycol, mono-stearate of ethylene glycol, the mono-stearate of triethylene glycol, the mono- or di-stearate of glycerol, triethanolamine stearate, diethanolamine stearate, mono ethanolamine stearate, ammonium oleate, ethylene glycol oleate, diethylene glycol oleate, triethylene glycol oleate, the mono- or di-oleate of glycerol, triethanolamine oleate, diethanolamine oleate, mono- 25 ethanolamine oleate or other like waxy bodies.

25 In place of or with the stearates and oleates above specified, the palmitic or other mono-fatty acid ethers or esters of glycols, polyglycols, glycerols and higher polyhydric alcohols may be 30 used.

35 The wax-like bodies may be used alone or in combination with such ingredients as cresylic acid, butyl acetate, polymerized fatty acid and glycero- or glyco-boric acid or cetyl alcohol or esters or ethers of higher fatty alcohols.

40 Beneficial results may be obtained by incorporating in the treating material mixtures of two or more of the above named or like ingredients as will be seen from a further description of my 45 invention.

45 For certain purposes it is advisable to add to any or a mixture of the above named wax-like bodies a proportion of the so-called non-emulsifiable wax-like bodies to act as sizes, hardeners, 50 etc. such as ceresin wax, beeswax, stearic acid, stearin, palmitic acid, ozokerite wax, carnauba wax, chlorinated naphthas and like bodies.

55 The wax-like body or mixture of such bodies may be added to the dope in amounts of 1% up

to 20%, preferably 3 to 7%, of the weight of the derivative of cellulose present, depending on the mixture used. Certain of the mixtures raise the viscosity of the dope to such an extent that heated filtration is required. The percent of the wax-like material to be added depends also on the solubility of the material in the dope and will vary with the process used.

By way of describing our invention still further and not with the intention of limiting its scope thereby, we give the following specific examples.

*Example I*

To a spinning solution of cellulose acetate in acetone there is added 5% diethylene glycol stearate based upon the weight of cellulose acetate. The diethylene glycol stearate is added in a hot solution of acetone. The dry spinning stability of the charge is good and may be spun to form yarn of 150 denier 40 filaments. The cross section of the filaments is 100% bulbous and of a squat type. The yarn spun has a very slightly subdued lustre and an appearance much like that of real silk.

25. The yarn delusters slightly in 30 minutes when treated with an aqueous solution containing 2 grams of soap per litre at 65° C. while yarn formed from a solution of cellulose acetate not containing the diethylene glycol stearate is not affected. When delustered for 30 minutes in an aqueous solution containing 2 grams of soap per liter at 95° C., it becomes very woolly and crinkled and delusters very heavily while a blank takes on a moderate delustre.

35

*Example II*

The process of Example I is carried out except that diethylene glycol oleate is used giving similar results.

40

*Example III*

The process of Example I is repeated except that distearate of glycerol is used giving approximately the same results.

45

*Example IV*

The process of Example II is repeated except that 5% of a mixture of equal parts of diethylene glycol stearate and triethanolamine stearate is used giving approximately the same results.

50 In all the processes of the above examples gave a filament of good cross-section and this is probably due to the wax-like body coming out of solution rapidly as the spinning thread cools due to the rapid evaporation of acetone or other solvent used in the dope.

It is to be understood that the foregoing de-

tailed description is given merely by way of illustration and that many variations may be made therein without departing from the spirit of our invention.

Having described our invention, what we desire to secure by Letters Patent is:

1. Yarns and staple fibres of cellulose acetate containing diethylene glycol stearate.

2. Artificial products having a basis of organic derivatives of cellulose and containing 10 wax-like higher fatty acid esters of polyhydric alcohols.

3. Yarns and staple fibres having a basis of organic derivatives of cellulose and containing 15 readily emulsifiable wax-like higher fatty acid esters of polyhydric alcohols.

4. Yarns and staple fibres having a basis of cellulose acetate and containing readily emulsifiable wax-like higher fatty acid esters of polyhydric alcohols.

5. Yarns and staple fibres having a basis of organic derivatives of cellulose and containing 20 higher fatty acid esters of diethylene glycol.

6. Yarns and staple fibres having a basis of cellulose acetate and containing higher fatty 25 acid esters of diethylene glycol.

7. Artificial products having a basis of organic derivatives of cellulose and containing wax-like compounds of higher fatty acids with polyhydric alcohols.

8. Staple fibres having a basis of organic derivatives of cellulose and containing wax-like compounds of higher fatty acids with polyhydric alcohols.

9. Artificial products having a basis of cellulose acetate and containing wax-like compounds 35 of higher fatty acids with polyhydric alcohols.

10. Staple fibres having a basis of cellulose acetate and containing wax-like compounds of higher fatty acids with polyhydric alcohols.

11. Artificial products having a basis of organic derivatives of cellulose and containing wax-like higher fatty acid esters of polyhydric alcohols, said esters containing only carbon, hydrogen and oxygen.

12. Yarns and staple fibres having a basis of organic derivatives of cellulose and containing readily emulsifiable wax-like higher fatty acid esters of polyhydric alcohols, said esters containing only carbon, hydrogen and oxygen.

13. Yarns and staple fibres having a basis of cellulose acetate and containing readily emulsifiable wax-like higher fatty acid esters of polyhydric alcohols, said esters containing only carbon, hydrogen and oxygen.

CAMILLE DREYFUS,  
WILLIAM WHITEHEAD.